

# UNITED STATES PATENT OFFICE.

CARLETON ELLIS, OF LARCHMONT, NEW YORK, ASSIGNOR TO ELLIS-FOSTER COMPANY,  
A CORPORATION OF NEW JERSEY.

## WOOD-OIL PUTTY.

1,029,800.

Specification of Letters Patent. Patented June 18, 1912.

No Drawing.

Application filed November 16, 1907. Serial No. 402,513.

To all whom it may concern:

Be it known that I, CARLETON ELLIS, a citizen of the United States, residing at Larchmont, in the county of Westchester 5 and State of New York, have invented certain new and useful Improvements in Wood-Oil Putty, of which the following is a specification.

This invention relates to putty; and comprises a dough-like plastic mass containing an inert mineral filler and a vehicle comprising sufficient wood oil to render the mass self-setting throughout, said putty remaining plastic until use and setting to a 15 firm mass after application without becoming brittle, friable and porous.

Putty as formerly made with linseed oil, has the disadvantage of gradually becoming a brittle mass which cracks and falls away 20 from the surface to which it has been applied. This is due largely to extreme oxidation of the linseed oil, which in its final stages gives rise to the formation of brittle resinous products. Linseed oil sets from within 25 out inwardly through oxidation, the degree of oxidation increasing with the time of exposure to air until the oil ultimately becomes converted into a resinous perishable mass. This oxidation is attended by and is dependent upon the production of porosity 30 during the oxidation.

My invention involves a putty made by the use of Chinese wood oil or similar self setting oil, such as Japanese wood oil, Han-kow oil, Tung oil; and the like, in combination with an extending oil such as mineral oil, and preferably with a resinous body such as colophonium. Wood oil on exposure 35 to air sets by a molecular change, the nature of which is obscure, and not primarily by oxidation. This setting is not attended with the production of pores. On admixture with mineral oils the setting is modified in some way and the compound vehicle thus 40 produced has setting properties which, I find, make it particularly adapted for the purposes of putty. The presence of rosin further advantageously affects this setting. This oily material is used as a basis with 45 50 which is incorporated an inert filler, such as whiting or other mineral powder or "thickener" used to give the necessary plasticity to the mass. Suitable inert mineral powders are whiting, ground lime-stone, includ-

ing dolomitic lime-stone, marble dust, alumina, magnesium carbonate, barytes, kaolin, talc, ground soap-stone, and the like.

Whatever inert filler is employed, it should be as finely powdered as possible and substantially free of grit and metallic particles. The ordinary uses of putty require that it be extremely fluent in order that it may properly fill cracks and crevices to which it is applied. The presence of even a small amount of gritty or metallic particles seriously affects the fluency of putty and may render the putty valueless.

I may also incorporate some oxidizable oils of a marked drying nature, including small proportions of linseed oil, or larger proportions of semi-drying oils, such as corn oil. Thus it becomes possible to produce compositions comprising a plurality of oils or drying oils including wood oil.

An illustrative formula representing the composition which I now consider the preferred embodiment of this invention, is made by melting twenty-five parts of rosin and adding thereto sixty parts of mineral oil having a specific gravity of about .865, and fifteen parts of Chinese wood oil. When this oil stock is thoroughly blended by suitable heating, it may be mixed with five hundred parts of a mixture of twenty parts of barytes and eighty parts whiting. The mixture is thoroughly ground together, preferably by trituration in a "chaser" or edge runner.

The proportions given in the above formula may, of course, be varied more or less to produce putties having different degrees of plasticity.

The use of wood oil as well as rosin in this composition gives rise to a highly coherent putty and this peculiar cohesiveness makes the material unusually plastic and resistant to weathering action. Under the influence of light and exposure, and in presence of the other materials mentioned, the wood oil changes to a polymeric form with possibly the formation of some eleomargaric acid, and in this polymerized form it gives to the putty for an indefinitely long time after application, a solidity, firmness, density, strength, elasticity and tenacity not found in putty made with the ordinarily used oils. Wood oil therefore produces a putty having properties differing from and

enormously superior to linseed oil putties, or putties, the vehicle of which consists of mineral oil and linseed oil in admixture.

The drying of the putty or what in this case may be termed the "setting", occurs throughout the entire mass almost simultaneously and yet the putty does not at any time adhere so firmly to the surfaces to which it may be applied, but that it may be removed with little difficulty whenever desired by the application of a putty knife or a scraping tool.

Another illustrative formula comprises 20 parts of wood oil, 60 parts of paraffin oil, 15 20 parts of rosin and 420 parts of China clay. The rosin may be omitted or replaced by the mineral oil.

A very desirable composition may be made by mixing 20 parts of wood oil with 20 80 parts of mineral oil or equivalent oily material having little or no real drying properties, and grinding this oil stock with 400 parts of a mineral thickener such as whiting. By varying the proportion of 25 wood oil, varying "setting" speeds may be obtained. Unlike linseed oil and mineral oil mixtures, wood oil confers upon the putty highly desirable properties, which render its adaptation to this art, of unusual 30 value.

I have observed when using whiting as the filler or thickener that red oil, or commercial oleic acid, or even palmitic and stearic acids act as assistants to the wood oil, 35 in securing a perfect blend and coherency. It is possible that the formation of a lime soap occurs to some extent in this case under the mechanical operation of grinding. A formula containing red oil comprises:—

|    |             |           |
|----|-------------|-----------|
| 40 | Wood oil    | 10 parts. |
|    | Red oil     | 5 "       |
|    | Mineral oil | 65 "      |
|    | Corn oil    | 20 "      |
| 45 | Whiting     | 400 "     |

The oils used may be subjected to the action of sulfur chlorid to impart greater viscosity. For example, 18 parts by volume of mineral oil of about .865 gravity may be 50 mixed with 2 parts each of corn oil and sulfur chlorid, and allowed to stand twenty-four hours. Eighteen parts by weight of this oil mixture may be mixed with eighty parts by weight of whiting and mixed for

a short time when two parts of wood oil are 55 added and the composition well ground in an edge runner.

What I claim is:

1. A self-setting putty comprising an inert pulverulent mineral filler in predominating amount, said filler consisting mainly of whiting, and being substantially free of metallic particles and a vehicle comprising wood oil in sufficient amount to cause the composition to be self-setting throughout. 65

2. As a self-setting putty, a plastic, doughlike composition comprising wood oil and an inert filler consisting mainly of whiting, and being substantially free of metallic particles, said wood oil being in amount 70 sufficient to cause the composition to be self-setting.

3. As a self-setting putty, a plastic, doughlike composition comprising wood oil, mineral oil and an inert filler comprising a 75 substantial amount of whiting, and being substantially free of metallic particles, said wood oil being in amount sufficient to cause the composition to be self-setting.

4. A putty consisting of a plastic doughlike composition comprising mineral oil, rosin, wood oil and a finely powdered mineral thickener. 80

5. A putty consisting of a plastic doughlike composition comprising as the oil stock, 85 about eighty (80) parts of mineral oil, and about twenty (20) parts of wood oil; and as the mineral thickener, about four hundred (400) parts of whiting.

6. A putty consisting of plastic doughlike composition comprising mineral oil, rosin, wood oil and a finely powdered mineral thickener containing whiting. 90

7. A putty consisting of a plastic doughlike composition comprising mineral oil, a 95 resinous body, wood oil and a finely powdered mineral thickener.

8. A putty consisting of a plastic doughlike composition comprising a non-drying oil, a plurality of oils having drying properties, including wood oil, and a thickener, 100 including whiting.

In testimony whereof I have affixed my signature in presence of two witnesses.

CARLETON ELLIS.

Witnesses:

NATHANIEL L. FOSTER,  
HENRIETTA BERKWITZ.